



US006946201B2

(12) **United States Patent**  
Preikschat et al.

(10) Patent No.: **US 6,946,201 B2**  
(45) Date of Patent: **Sep. 20, 2005**

(54) **CHROMIUM (VI)-FREE CONVERSION LAYER AND METHOD FOR PRODUCING IT**

2,035,385 A 3/1936 McLean  
2,106,904 A 2/1938 Wilhelm

(Continued)

(75) Inventors: **Patricia Preikschat**, Trebur (DE); **Rolf Jansen**, Trebur (DE); **Peter Hulser**, Trebur (DE)

FOREIGN PATENT DOCUMENTS

(73) Assignee: **SurTec International GmbH**, Zwingenberg (DE)

DE 21 66737 A1 6/1975  
DE 29 00 099 B2 7/1981  
DE 30 38 699 A1 7/1981  
DE 32 13 384 A1 12/1982  
DE 34 23 990 A1 1/1985  
DE 32 13 384 C2 1/1991  
DE 41 35 524 A1 4/1993

(Continued)

(\*) Notice: Subject to any disclaimer, the term of this patent is extended or adjusted under 35 U.S.C. 154(b) by 197 days.

OTHER PUBLICATIONS

(21) Appl. No.: **09/904,993**

“Kinetics of Formation and Dissociation of [Cr30(02CCH3)6(urea)3]+: An Example of Statistically Controlled Kinetics and Equilibrium,” John P. Bourke, et al., Inorganic Chemistry; vol. 35, No. 6, Mar. 13, 1996; pp. 1577–1581.\*

(22) Filed: **Jul. 13, 2001**

“Electrodeposited Coatings of Zinc on Iron or Steel: Concepts, Corrosion Testing and Corrosion Resistance,” DIN 50961; Sep. 2000; pp. 1–6 (translation).\*

(65) **Prior Publication Data**

“Galvanische Überzüge; Zink- und Cadmiumüberzüge auf Eisenwerkstoffen; Chromatierung der Zink- und Cadmiumüberzüge,” DIN 50961; Jun. 1987; pp. 4 and 5 (original and translation).\*

US 2003/0207133 A1 Nov. 6, 2003

(Continued)

**Related U.S. Application Data**

Primary Examiner—Robert R. Koehler

(63) Continuation of application No. 09/171,558, filed as application No. PCT/DE97/00800 on Apr. 18, 1997, now Pat. No. 6,287,704.

(74) Attorney, Agent, or Firm—Pearne & Gordon LLP

(30) **Foreign Application Priority Data**

**ABSTRACT**

Apr. 19, 1996 (DE) ..... 196 15 664

A chromium(VI)-free, chromium(III)-containing and substantially coherent conversion layer on zinc or zinc alloys presenting, even in the absence of further components such as silicate, cerium, aluminum and borate, a corrosion protection of approx. 100 to 1000 h in the salt spray test according to DIN 50021 SS or ASTM B 117-73 until first attack according to DIN 50961 Chapter 10; being clear, transparent and substantially colorless and presenting multi colored iridescence; having a layer thickness of approx. 100 nm to 1000 nm; and being hard, adhering well and being resistant to wiping.

(51) **Int. Cl.<sup>7</sup>** ..... B32B 15/04; C23C 22/30  
(52) **U.S. Cl.** ..... 428/472.1; 148/247; 148/251;  
148/258; 148/265; 148/267; 148/268; 148/273;  
148/274; 148/283; 148/284; 427/430.1;  
427/435; 428/628; 428/629; 428/632; 428/658;  
428/659

(58) **Field of Search** ..... 428/472.1, 628,  
428/629, 632, 658, 659; 427/430.1, 435;  
148/247, 251, 258, 265, 267, 268, 273,  
274, 283, 284; 106/14.21

(56) **References Cited**

**78 Claims, 38 Drawing Sheets**

**U.S. PATENT DOCUMENTS**

2,035,380 A 3/1936 Wilhelm



Computer simulation of the kinetic model of chromate coating of zinc for various rate constants

## U.S. PATENT DOCUMENTS

|              |           |                        |           |
|--------------|-----------|------------------------|-----------|
| 2,559,878 A  | 7/1951    | Johnson                |           |
| 2,563,431 A  | 8/1951    | Spruance, Jr.          |           |
| 2,620,265 A  | 12/1952   | Hesch                  |           |
| 2,904,413 A  | 9/1959    | Hampel                 |           |
| 3,072,516 A  | 1/1963    | Bellinger et al.       |           |
| RE26,130 E   | 12/1966   | Bellinger et al.       |           |
| 3,382,111 A  | 5/1968    | Tongyai et al.         |           |
| 3,477,882 A  | 11/1969   | Coulman                |           |
| 3,553,034 A  | 1/1971    | Harvey et al.          |           |
| 3,556,868 A  | 1/1971    | Ziemba                 |           |
| 3,787,326 A  | 1/1974    | Deyrup                 |           |
| 3,843,430 A  | 10/1974   | Kinder .....           | 252/79.3  |
| 3,857,739 A  | 12/1974   | Prust et al.           |           |
| 3,900,689 A  | 8/1975    | Deyrup                 |           |
| 3,932,198 A  | 1/1976    | Schneider              |           |
| 4,126,490 A  | 11/1978   | Aoki                   |           |
| 4,141,758 A  | 2/1979    | Glassman et al.        |           |
| 4,169,741 A  | 10/1979   | Lampatzer et al.       |           |
| 4,171,231 A  | 10/1979   | Bishop et al.          |           |
| 4,263,059 A  | 4/1981    | Guhde et al.           |           |
| 4,298,404 A  | 11/1981   | Greene .....           | 148/247   |
| 4,349,392 A  | 9/1982    | Huvar                  |           |
| 4,359,345 A  | 11/1982   | DaFonte, Jr.           |           |
| 4,359,346 A  | 11/1982   | DaFonte, Jr.           |           |
| 4,359,347 A  | 11/1982   | DaFonte, Jr.           |           |
| 4,359,348 A  | 11/1982   | Crotty                 |           |
| 4,367,099 A  | 1/1983    | Lash et al.            |           |
| 4,384,902 A  | 5/1983    | Crotty et al.          |           |
| 4,444,601 A  | 4/1984    | Greene .....           | 428/658   |
| 4,539,348 A  | 9/1985    | Gajria et al.          |           |
| 4,578,122 A  | 3/1986    | Crotty                 |           |
| 4,705,576 A  | 11/1987   | Klos et al.            |           |
| 4,749,418 A  | 6/1988    | Saeki et al.           |           |
| 4,801,337 A  | 1/1989    | Higgins .....          | 148/267   |
| 5,091,023 A  | 2/1992    | Saeki et al.           |           |
| 5,141,575 A  | 8/1992    | Yoshitake et al.       |           |
| 5,230,750 A  | 7/1993    | Shindou et al.         |           |
| 5,368,655 A  | * 11/1994 | Klos .....             | 148/267   |
| 5,393,354 A  | 2/1995    | Bishop                 |           |
| 5,407,749 A  | 4/1995    | Bishop                 |           |
| 5,415,702 A  | 5/1995    | Bishop et al.          |           |
| 5,807,442 A  | 9/1998    | Goodreau               |           |
| 5,820,741 A  | 10/1998   | Bibber .....           | 205/287   |
| 5,876,517 A  | 3/1999    | Jeannier .....         | 148/264   |
| 6,287,704 B1 | * 9/2001  | Preikschat et al. .... | 428/472.1 |
| 6,375,726 B1 | 4/2002    | Matzdorf et al. ....   | 148/247   |

## FOREIGN PATENT DOCUMENTS

|    |              |         |
|----|--------------|---------|
| EP | 0 034 040 A1 | 8/1981  |
| EP | 0 034 040 A1 | 9/1981  |
| EP | 0 337 411 A2 | 10/1989 |
| EP | 0 337 411 B1 | 10/1989 |
| GB | 14 61 244    | 1/1977  |
| GB | 2 097 024 A  | 10/1982 |
| GB | 2097024 A    | 10/1982 |
| GB | 2 144 773 A  | 3/1985  |
| JP | 50-1934      | 1/1975  |
| JP | 61-587       | 1/1986  |
| RU | 1781316 A1   | 12/1992 |

## OTHER PUBLICATIONS

Dr.-Ing. Uka Handreg and Dipl.-Ing. Stefen Piepenstock, *Prüfbericht—Untersuchungen an Blauchromatierungen*, Jan. 8, 2002, pp. 1–4.

Dipl.-Ing. Britta Schlüter, *Prüfbericht—Untersuchungen an Blauchromatierungen*, Jun. 19, 2002, pp. 1–3.

Von W. Stechelbach, *Chromatierungstechnik an Verzinkten Oberflächen*, Galvanotechnik, D–7968 Saulgau, 82 (1991) Nr. 8, pp. 2669–2672, no month given.

*Zusammenstellung der Experimentellen Daten*, Jul. 17, 2002, 9 pages.

SurTec® 660 *Dreiwertige Blauchromatierung*, SurTec GmbH, Feb. 1994.

SurTec® 662 *Dreiwertige Temperbeständige Blauchromatierung*, SurTec GmbH, Feb. 1994.

SurTec® 664 *Dreiwertige, Temperbeständige Blauchromatierung Mit Eiseninhibitor*, SurTec GmbH, Feb. 1994.

Optische Defizite der Surtec Beispiele 2 und 3 aus dem Patent EP 0 907 762, at least as early as Jul. 17, 2002.

Chemisch erzeugte Schutzschichten, pp. 470–473, at least as early as Jul. 22, 2002.

Coventya, *Internal Note*, Subject: Opposition au brevet EP 907762, Jul. 1, 2002, 4 pages.

Peter Hülser, et al., *Chromatierung*, Mo Metalloberfläche Beschichten von Metall Und Kunststoff, Oct. 1996, 5 pages.

“Some Metal Derivatives of Azo and Azomethine Dyes”, Journal of the American Chemical Society, vol. 74, No. 14, Jul. 20, 1952, pp. 3461 and 3509–3512.

Database WPI, Section Ch, Week 9402, Derwent Publications Ltd., London, GB; AN 94–014365, XP002038536 & SU 1 781 316 A (Magn Mining Metal Inst), Dec. 15, 1992, siehe Zusammenfussung.

PCT International Search Report for PCT International Application PCT/DE97/00800, Sep. 5, 1997.

“Chromate Coating From Trivalent Solution,” Products Finishing, Aug., 1983, pp. 64–65.

Barnes, et al., “Non-Chromate Passivation Treatments For Zinc,” Transactions of the Institute of Metal Finishing, Summer, 1982, pp. 45–48, vol. 60.

Klos, “Clear Chromates: Theory and Practice,” Products Finishing, Jun., 1988, pp. 72–78.

DIN 50 961, Ch. 10, “Prüfung des Chromatierüberzuges” (English Title “Testing of Chromate Conversion Coatings”), Jun. 1987 (with English translation).

Arthur Schaier, First Request For Reexamination of U.S. patent No. 6,287,704 (granted as re-exam Ser. No. 90/006, 211), Request filed in U.S. Patent Office on Jan. 25, 2002, pp. 1–118.

Arthur Schaier, Submission of Prior Art Under 37 CFR 1.501 filed in re-exam proceeding Ser. No. 90/006,211, filed in U.S. Patent Office on Mar. 11, 2002, pp. 1–4.

Patricia Preikschat, Declaration of Patricia Preikschat Udner Rule 1.132 filed in re-exam proceeding Ser. No. 90/006,211, dated Dec. 4, 2002, pp. 1–10.

Arthur Schaier, Second Request For Reexamination of U.S. patent No. 6,287,704 (granted as re-exam Ser. No. 90/006, 672), filed in U.S. Patent Office on Jun. 20, 2003, pp. 1–25.

Sudha Damji, Declaration of Sudha Damji and attached Exhibit A, dated Jun. 18, 2003, (submitted with the second request for reexamination of U.S. patent No. 6,287,704), filed in re-exam proceeding Ser. No. 90/006,672 on Jun. 20, 2003, pp. 1–33.

\* cited by examiner

Fig. 1

Color comparison of various passive layers



Substrate: Zinc-plated screws

|                    |                    |
|--------------------|--------------------|
| Blue chromation:   | Left picture half  |
| Invention:         | Center             |
| Yellow chromation: | Right picture half |



FIG. 2

Fig. 3

Bandwidth of iridescence according to the present invention  
(on zinc-plated screws)



Fig. 4

Comparison test with EP 0 034 040

Example 16

Example 17



The upper picture half, one the outer left and right, shows a black cloth whereby the abrasions on the metal sheets shown in the top picture half were obtained. Layer portions - discernible as whitish stains - are on both pieces of cloth. The lower picture half shows the unmarred layers of the prior art.

Substrate: Zinc-plated steel sheet.

Fig. 5  
Pattern 1, Measurement Position A

Fig. 6  
Pattern 1, Measurement Position A





Fig. 8  
Sample 1, Measurement Position B



Fig. 9

Sample 2, Measurement Position A



Fig. 10  
Sample 2, Measurement Position A

**Fig. 11**  
**Sample 2, Measurement Position B**



Fig. 12  
Sample 2, Measurement Position B



Fig. 13

Sample 3, Measurement Position A



Fig. 14  
Sample 3, Measurement Position A



Fig. 15

Sample 4, Measurement Position A



Fig. 16  
Sample 4, Measurement Position A



Fig. 17

Sample 6, Measurement Position A



Fig. 18  
Sample 5, Measurement Position A



Fig. 19

Sample 6, Measurement Position A



Fig. 20  
Sample 6, Measurement Position A



Fig. 21

Sample 6, Measurement Position B



Fig. 22  
Sample 6, Measurement Position B



Fig. 23

Sample 6, Measurement Position C



Fig. 24  
Sample 6, Measurement Position C



Fig. 25  
Sample 6, Measurement Position D



Fig. 26



Fig. 27  
Sample 7, Measurement Position A



Fig. 28



Fig. 29

Sample 7, Measurement Position B



Fig. 30

Sample 7, Measurement Position B



Fig. 31

### Sample 8, Measurement Position A



Fig. 32

Sample 8, Measurement Position A



Fig. 33

Sample 9, Measurement Position A



Fig. 34

Sample 9, Measurement Position A



Fig. 35

Sample 9, Measurement Position B



Fig. 36  
Sample 9, Measurement Position B



FIG. 37

|                                              |     | Methods            |           |                                             |             |                                |               |            |
|----------------------------------------------|-----|--------------------|-----------|---------------------------------------------|-------------|--------------------------------|---------------|------------|
|                                              |     | Ellipsometry<br>nm | SEM<br>nm | Glow-discharge spectrometer<br>nm (Cr > 1%) | with Cr (%) | chromium index<br>nm (Cr > Zn) | nm (Cr > 30%) | Sample No. |
| <b>1. Prior Art</b>                          |     |                    |           |                                             |             |                                |               |            |
| Yellow chromation<br>Cr(III) + Cr(VI)        | -   | 300                | 440       | 11                                          | 48          | 17                             | 25            | 9          |
| Blue chromation<br>Cr(III)                   | 98  | 60                 | 60        | 8                                           | 5           | 0                              | 0             | 8          |
| <b>2. Invention (Chromitiation)</b>          |     |                    |           |                                             |             |                                |               |            |
| 60 °C<br>Cr(III)                             | 432 | 300                | 344       | 7                                           | 23          | 2                              | 15            | 1,2,3,4,5  |
| 100 °C<br>Cr(III)                            | 595 | -                  | 358       | 10                                          | 38          | 22                             | 28            | 6          |
| 60 °C on Zn/Fe<br>Cr(III)                    | -   | -                  | 282       | 6                                           | 16          | 0                              | 16            | 7          |
| 100 °C, two-fold<br>concentration<br>Cr(III) | 953 | -                  | -         | -                                           | -           | -                              | -             | -          |

Fig. 38



Computer simulation of the kinetic model of chromate coating of zinc for various rate constants

## 1

CHROMIUM (VI)-FREE CONVERSION  
LAYER AND METHOD FOR PRODUCING ITCROSS-REFERENCE TO RELATED  
APPLICATIONS

This application is a continuation of U.S. patent application Ser. No. 09/171,558 filed on Mar. 29, 1999, now U.S. Pat. No. 6,287,704, which is a § 371 of PCT Application Ser. No. PCT/DE97/00800 filed Apr. 18, 1997.

## FIELD OF THE INVENTION

The present invention relates to chromium(VI)-free, chromium(III)-containing, substantially coherent conversion layers, a method for producing them, a concentrate, a passivation bath, a passivating method, a passive layer, and a conversion layer.

## BACKGROUND OF THE INVENTION

Metallic materials, in particular iron and steel, are plated with zinc or cadmium in order to protect them from corrosive environmental influences. The corrosion protection of zinc resides in the fact that it is even less precious than the base metal and therefore at first exclusively draws the corrosive attack; it acts as a sacrificial layer. The base metal of the respective zinc-plated component remains unimpaired as long as it is continuously covered with zinc, and the mechanical functionality remains preserved over longer periods of time than in the case of parts not plated with zinc. Thicker zinc layers naturally afford higher corrosion protection than thin layers inasmuch as corrosive erosion of thicker layers simply takes more time.

The corrosive attack on the zinc layer, in turn, can be greatly delayed by application of a chromation, or chromate coating, whereby corrosion of the base metal is even further postponed than by mere zinc plating. A considerably better corrosion protection is afforded by the zinc/chromate layer system than by a mere zinc layer of identical thickness. Moreover by means of chromation the optical deterioration of a component due to environmental influences is further postponed—the corrosion products of zinc, referred to as “white rust”, equally interfere with the optical appearance of a component.

The advantages of an applied chromation are so important that almost any galvanically zinc-plated surface is in addition chromate coated as well. The prior art knows four chromations named after their colorations, which are each applied by treating (immersion, spraying, rolling) a zinc-plated surface with the corresponding aqueous chromate coating solution. Moreover yellow and green chromations for aluminum are known which are produced analogously. In any case, these are variously thick layers of substantially amorphous zinc/chromium oxide (or aluminum/chromium oxide) with non-stoichiometric compositions, a certain water content, and inserted foreign ions. These are known and classified into method groups in accordance with German Industrial Standard (DIN) 50960, Part 1:

## 1) Colorless and blue chromations, Groups A and B

The blue chromate layer has a thickness of up to 80 nm, is weakly blue in its inherent color and presents a golden, reddish, bluish, greenish or yellow iridescent coloring brought about by refraction of light in accordance with layer thicknesses. Very thin chromate layers lacking almost any inherent color are referred to as colorless chromations (Group A). The chromate coating solution may in either case consist of hexavalent as well as trivalent chromates and

## 2

mixtures of both, moreover conducting salts and mineral acids. There are fluoride-containing and fluoride-free variants. Application of the chromate coating solutions is performed at room temperature. The corrosion protection of unmarred blue chromations amounts to 10–40 h in the salt spray cabinet according to DIN 50021 SS until the first appearance of corrosion products. The minimum requirement for Method Groups A and B according to DIN 50961 Chapter 10 Table 3 is 8 h for drumware and 16 h for shelfware.

## 2) Yellow Chromations, Group C

The yellow chromate layer has a thickness of approx. 0.25–1  $\mu\text{m}$ , a golden yellow coloring, and frequently a strongly red-green iridescent coloring. The chromate coating solution substantially consists of hexavalent chromate, conducting salts and mineral acids dissolved in water. The yellow coloring is caused by the significant proportion (80–220 mg/m<sup>2</sup>) of hexavalent chromium which is inserted besides the trivalent chromium produced by reduction in the course of the layer formation reaction. Application of the chromate coating solutions is performed at room temperature. The corrosion protection of unmarred yellow chromations amounts to 100–200 h in the salt spray cabinet according to DIN 50021 SS until the first appearance of corrosion products. The minimum requirement for Method Group C according to DIN 50961 Chapter 10 Table 3 amounts to 72 h for drumware and 96 h for shelfware.

## 3) Olive Chromations, Group D

The typical olive chromate layer has a thickness of up to 1.5  $\mu\text{m}$  and is opaquely olive green to olive brown. The chromate coating solution substantially consists of hexavalent chromate, conducting salts and mineral acids dissolved in water, in particular phosphates or phosphoric acid, and may also contain formates. Into the layer considerable amounts of chromium(VI) (300–400 mg/m<sup>2</sup>) are inserted. Application of the chromate coating solutions is performed at room temperature. The corrosion protection of unmarred olive chromations amounts to 200–400 h in the salt spray cabinet according to DIN 50021 SS until the first appearance of corrosion products. The minimum requirement for Method Group D according to DIN 50961 Chapter 10 Table 3 is 72 h for drumware and 120 h for shelfware.

## 4) Black Chromations, Group F

The black chromate layer is fundamentally a yellow or olive chromation having colloidal silver inserted as a pigment. The chromate coating solutions have about the same composition as yellow or olive chromations and additionally contain silver ions. With a suitable composition of the chromate coating solution on zinc alloy layers such as Zn/Fe, Zn/Ni or Zn/Co, iron, nickel or cobalt oxide will be incorporated into the chromate layer as a black pigment so that silver is not required in these cases. Into the chromate layers considerable amounts of chromium(VI) are inserted, namely between 80 and 400 mg/m<sup>2</sup> depending on whether the basis is a yellow or olive chromation. Application of the chromate coating solutions is performed at room temperature. The corrosion protection of unmarred black chromations on zinc amounts to 50–150 h in the salt spray cabinet according to DIN 50021 SS until the first appearance of corrosion products. The minimum requirement for Method Group E according to DIN 50961 Chapter 10 Table 3 is 24 h for drumware and 48 h for shelfware. Black chromations on zinc alloys are considerably above the specified values.

## 5) Green Chromations for Aluminum, Group E

The green chromation on aluminum (known under the name of aluminum green) is of a matt green and not iridescent. The chromate coating solution substantially con-

sists of hexavalent chromate, conducting salts and mineral acids dissolved in water as well as particularly phosphates and silicofluorides. Contrary to a prevailing opinion the formed chromate/phosphate layer is, as evidenced by iodised starch tests, not always 100% chromium(VI)-free. The production of aluminum green in chromate coating solutions exclusively on the basis of chromium(III) is not known.

In accordance with the prior art, thick chromate layers affording high corrosion protection >100 h in the salt spray cabinet according to DIN 50021 SS or ASTM B 117-73 until the appearance of first corrosion products according to DIN 50961 (June 1987) Chapter 10, in particular Chapter 10.2.1.2, in the absence of sealing or any other particular aftertreatment (DIN 50961, Chapter 9) may only be produced by treatment with dissolved, markedly toxic chromium(VI) compounds. Accordingly the chromate layers having the named requirements to corrosion protection still retain these markedly toxic and carcinogenic chromium(VI) compounds, which are, moreover, not entirely immobilised in the layer. Chromate coating with chromium(VI) compounds is problematic with respect to workplace safety. Use of zinc-plated chromations produced with chromium(VI) compounds, such as the widespread yellow chromations e.g. on screws, constitutes a potential hazard to the population and increases the general cancer risk.

U.S. Pat. No. 4,384,902, in particular with Examples 1, 2, 4 and 5, describes conversion layers which satisfy the requirements in the salt spray test. In all of the cases, these are cerium-containing layers presenting a yellowish coloration which is accentuated by the cerium(IV) ion. The examples only contain cerium(III), and hydrogen peroxide as an oxidant, in the bath solution. In the description it is set forth that hydrogen peroxide in the acidic medium does not represent an oxidant for Ce(III), however during deposition the pH value nevertheless rises so high at the surface that a sufficient amount of Ce(IV) may be generated. The yellowish coloration achieved by this bath composition indeed appears to indicate that an oxidation has taken place—however, only an oxidation from Ce(III) to Ce(IV). Tetravalent cerium is an even more powerful oxidant than hexavalent chromium, for which reason Ce(IV) will produce from Cr(III) the Cr(VI) which is to be avoided. Cr(VI) has a very strong yellow coloration and is known as an anticorrosion agent. The layer described in U.S. Pat. No. 4,384,902 is thus not free of hexavalent chromium.

#### BRIEF DESCRIPTION OF THE DRAWINGS

The file of this patent contains at least one drawing executed in color. Copies of this patent with color drawings will be provided by the Patent Office upon request and payment of the necessary fee.

FIG. 1 is a color comparison of various passive layers; it shows a comparison of the present invention with blue and yellow chromations. The substrate is zinc-plated screws. The left picture half is blue chromation; the center is the invention; the right picture half is yellow chromation.

FIG. 2 is a scanning electron microscope image (40,000H) showing a comparison of the present invention ("chromitization") with blue and yellow chromations. "Gelbchromatierung" means yellow chromation; "Chromitierung" means chromitization; "Blauchromatierung" means blue chromation; "Zink" means zinc.

FIG. 3 is a color photo showing the band width of the iridescent coloring in accordance with the present invention on zinc surfaces (zinc-plated screws);

FIG. 4, a comparison test with EP 0 034 040, shows coatings of the prior art in accordance with EP 0 034 040. Example 16 is on the left hand side, Example 17 is on the right hand side. The upper picture half, on the outer left and right, shows a black cloth whereby the abrasions on the metal sheets shown in the top picture half were obtained. Layer portions—discernible as whitish stains—are on both pieces of cloth. The lower picture half shows the unmarred layers of the prior art. The substrate is zinc-plated steel sheet.

FIGS. 5 to 36 show depth profile analyses of layers according to the invention and layers resulting from the conventional blue and yellow chromations, wherein the depth profile analyses were measured by glow-discharge spectrometry (spectrometer: JY5000RF);

FIG. 37 is a table containing the evaluation of the depth profile analyses of FIGS. 5 to 36.

FIG. 38 is a computer simulation of the kinetic model of chromate coating of zinc for various rate constants.

#### DETAILED DESCRIPTION OF THE PREFERRED EMBODIMENTS OF THE INVENTION

The layer according to the invention is, however, produced in the absence of any oxidant and consequently free of hexavalent chromium. This can in particular be seen from the fact that the layer according to the invention is not yellow.

Even where the yellow coloration and the enhanced corrosion protection should be brought about by nothing but Ce(IV), the layer according to the invention affords the desired corrosion protection even without this very costly and rare addition.

U.S. Pat. No. 4,359,348 also describes conversion layers which satisfy the above mentioned requirements in the salt spray test. These, too, in all cases are cerium-containing layers which present the yellowish coloration accentuated by the cerium(IV) ion. This document thus does not exceed U.S. Pat. No. 4,384,902.

It is therefore an object of the present invention to furnish a chromium(VI)-free, thick conversion layer having a high chromium content on zinc or zinc alloys.

For the purposes of the present inventions the applicant coined the term "chromitization" in order to clearly distinguish the present invention from the chromations which are customary in the prior art, and in order to make clear that neither the obtained conversion layer nor the compositions (concentrates/passivation baths) whereby the coatings according to the invention are produced contain the toxic chromium(VI), whereas the obtained corrosion protection nevertheless is superior to that of yellow chromation.

EP 00 34 040 A1 does describe a multiplicity of layers, of the larger group of which (produced under the standard conditions set forth by Barnes/Ward) the color is not specified, however referred to as clear. Two Examples, namely Nos. 16 and 17, describe a greenish borate-containing layer described as cloudy-dull to non-transparent.

Example 14 describes a layer affording a corrosion protection of only 4 hours.

Concerning the features of the invention, the following should be noted:

In glow-discharge spectrometry several elements could not be detected while others could not be calibrated. Therefore the chromium/(chromium+zinc) phases were compared to each other. The chromium index is the average chromium

## 5

content in the layer >1% Cr, multiplied by the layer thickness. The chromium index is proportional to the chromium quantity on the surface (mg/m<sup>2</sup>).

Further advantages and features of the present invention result from the description of embodiments and from theoretical reflections which are not binding on the one hand and were, on the other hand, carried out by the inventors while having knowledge of the present invention, and by referring to the drawings.

The conversion layer preferably has a layer thickness of about 100 to 1000 nm, the conversion layer having across the conversion layer thickness a chromium content of greater than 1% based upon zinc and chromium, the conversion layer having an average chromium content of more than approximately 5% based on zinc and chromium, and the conversion layer having a chromium index greater than approximately 10, wherein the chromium index is defined as the average chromium content (chromium/(chromium+zinc)) in the layer greater than 1% Cr, multiplied by the layer thickness in nm.

Preferably the conversion layer has a chromium-rich zone greater than approximately 20% chromium, based upon zinc and chromium in the conversion layer, of more than approximately 15 nm.

The conversion layer may be transparent, clear, or substantially colorless. The conversion layer may be iridescent, and may present multi-colored iridescence.

For enhanced corrosion protection the conversion layer may additionally contain one or more components selected from the group consisting of silicate, cerium, aluminum, and borate. The conversion layer may contain cobalt or one or more metal compounds having valences of 1 to 6. The conversion layer may include one or more metal compounds selected from the group consisting of Na, Ag, Al, Co, Ni, Fe, Ga, In, La, Ce, Pr, Nd, Pm, Sm, Eu, Gd, Tb, Dy, Ho, Er, Tm, Yb, Lu, Zr, Sc, Ti, V, Cr, Mn, Cu, Zn, Y, Nb, Mo, Hf, Ta, and W.

The conversion layer may include one or more ions selected from the group consisting of anions and may include one or more ions selected from the group consisting of halide ions, sulfurous ions, nitrate ions, phosphorus-containing ions, carboxylic acid anions, and silicon-containing anions.

The conversion layer may include one or more ions selected from the group consisting of chloride ions, sulfate ions, phosphate ions, diphosphate ions, linear and cyclic oligophosphate ions, linear and cyclic polyphosphate ions, hydrogen phosphate ions, and silicate anions.

The conversion layer may include one or more materials selected from the group consisting of polymers, corrosion inhibitors, silicic acids, surfactants, polyols, organic acids, amines, plastics dispersions, dyes, pigments, chromogenic agents, amino acids, siccatives, and dispersing agents.

The conversion layer may include one or more materials selected from the group consisting of organic polymers, colloidal or disperse silicic acids, diols, triols, monocarboxylic acids, carbon black, metal chromogenic agents, glycin, and cobalt siccatives.

The conversion layer may include one or more materials selected from the group consisting of dyes and color pigments.

In a method according to the invention, a metallic surface preferably is treated with a solution of at least one chromium (III) complex and at least one salt, wherein chromium (III) is present in the solution in a concentration of approximately

## 6

5 to 100 g/l; and the chromium (III) complex has ligand replacement kinetics more rapid than the fluoride replacement kinetics in chromium (III)-fluorocomplexes. This method produces a chromium (VI)-free conversion layer affording at least the corrosion protection of conventional chromium (VI)-containing yellow chromations.

Metallic surfaces suitable for application of the conversion layer include zinc, zinc alloy, and zinc alloy with iron.

In the method the treating is preferably carried out at an elevated temperature, or at a temperature of 20–100° C., more preferably 20–80° C., more preferably 30–60° C., more preferably 40–60° C.

In the method the chromium (III) complex preferably has chelate ligands which are selected from the group consisting of dicarboxylic acids, tricarboxylic acids, hydroxycarboxylic acids, acetylacetone, urea, urea derivatives, mixtures thereof, among each other as well as in mixed complexes with inorganic anions and H<sub>2</sub>O.

In the method the chromium (III) complex preferably has chelate ligands which are selected from the group consisting of oxalic, malonic, succinic, glutaric, adipic, pimelic, suberic, azelaic and sebatic acids, mixtures thereof, and in mixed complexes with inorganic anions and H<sub>2</sub>O.

In the method the chromium (III) complex preferably has chelate ligands which are selected from the group consisting of maleic acid, phthalic acid, terephthalic acid, tartaric acid, citric acid, malic acid, ascorbic acid, mixtures thereof, and in mixed complexes with inorganic anions and H<sub>2</sub>O.

In the method the chromium (III) complex preferably has chelate ligands which are selected from the group consisting of malonic acid and malonic acid in mixed complexes with inorganic anions and H<sub>2</sub>O.

The method may be performed repeatedly on the metallic surface.

In the method the treating may be carried out at a temperature of 20 to 100° C. with rinsing water recycling over at least 2 cascaded rinsing stages; a blue chromation may be performed in one of the rinsing stages.

The method may include an immersion period of between approximately 15 and 200 seconds or of between approx. 15 and 100 seconds or an immersion period of approx. 30 seconds.

A passivation bath for passivating a metal surface preferably comprises chromium (III) in a concentration of approximately 5 to 100 g/l; the chromium (III) being present in the bath in the form of at least one chromium (III) complex having ligand replacement kinetics more rapid than the fluoride replacement kinetics in chromium (III)-fluorocomplexes. The bath preferably substantially contains chromium (III) as a passivating component.

The chromium (III) complex in the bath preferably is selected from complexes with chromium (III) and at least one chelate ligand selected from the group consisting of dicarboxylic acids, tricarboxylic acids, hydroxycarboxylic acids, acetylacetone, urea, urea derivatives, mixtures thereof, among each other as well as in mixed complexes with inorganic anions and H<sub>2</sub>O.

The chromium (III) complex in the bath may be selected from complexes with chromium(III) and at least one chelate ligand selected from the group consisting of oxalic, malonic, succinic, glutaric, adipic, pimelic, suberic, azelaic and sebatic acids, mixtures thereof, and in mixed complexes with inorganic anions and H<sub>2</sub>O.

The chromium (III) complex in the bath may be selected from complexes with chromium(III) and at least one chelate

7

ligand selected from the group consisting of maleic acid, phthalic acid, terephthalic acid, tartaric acid, citric acid, malic acid, ascorbic acid, mixtures thereof, and in mixed complexes with inorganic anions and H<sub>2</sub>O.

The chromium (III) complex in the bath may be selected from complexes with chromium(III) and at least one chelate ligand selected from the group consisting of malonic acid and malonic acid in mixed complexes with inorganic anions and H<sub>2</sub>O.

The bath may also include one or more components selected from the group consisting of scalers, dewatering fluids, additional metal compounds, anions, polymers, corrosion inhibitors, silicic acids, surfactants, polyols, organic acids, amines, plastics dispersions, dyes, pigments, chromogenic agents, amino acids, siccatives and dispersing agents. The bath may also include one or more components selected from the group consisting of 1- to 6-valent metal compounds, halide ions, sulfurous ions, nitrate ions, phosphoric ions, carboxylic acid anions, silicon-containing anions, organic polymers, colloidal or disperse silicic acids, diols, triols, monocarboxylic acids, carbon black, metallic chromogenic agents, glycine, and cobalt siccatives. The bath may also include one or more components selected from the group consisting of metal compounds of Na, Ag, Al, Co, Ni, Fe, Ga, In, La, Ce, Pr, Nd, Pm, Sm, Eu, Gd, Th, Dy, Ho, Er, Tm, Yb, Lu, Zr, Sc, Ti, V, Mn, Cu, Zn, Y, Nb, Mo, Hf, Ta, and W, chloride ions, sulfate ions, phosphate ions, diphosphate ions, linear and cyclic oligophosphate ions, linear and cyclic polyphosphate ions, hydrogen phosphate ions and silicate anions.

Chromium (III) is preferably present in the bath in a concentration of approximately 5 g/l to 80 g/l, more preferably approximately 5 g/l to 60 g/l, more preferably approximately 10 g/l to 30 g/l, more preferably approximately 20 g/l. The bath preferably has a pH between approximately 1.5 and 3, more preferably approximately 2 to 2.5. The temperature of the bath is preferably approx. 20 to 100° C., more preferably approximately 20 to 80° C., more preferably approximately 30 to 60° C., more preferably approx. 40 to 60° C.

To facilitate preparation of a passivation solution, a concentrate may be prepared. The concentrate preferably substantially contains chromium (III) for a passivating component, wherein the chromium (III) is present in the form of at least one complex having ligand replacement kinetics more rapid than the fluoride replacement kinetics in chromium (III)-fluorocomplexes. The concentrate is preferably in either liquid or solid form. The concentrate may be used for producing a passivation solution for passivating a metal surface such as a metal surface selected from the group consisting of zinc, cadmium, aluminum and alloys of these metals among each other and/or with iron or other metals.

#### EXAMPLE 1

The following experiment was carried out:

Small steel parts were bright-zinc coated electrolytically (approx. 15 μm) and, following galvanisation, singly immersed in a boiling (approx. 100° C.), aqueous solution containing:

8

100 g/l CrCl<sub>3</sub>·6 H<sub>2</sub>O (trivalent chromium salt)

100 g/l NaNO<sub>3</sub>

15.75 g/l NaF

26.5 g/l citric acid·1 aq

which had previously been adjusted to a pH value of 2.5 with sodium hydroxide solution. The immersion time was 30 s.

10 The parts were then rinsed with water and dried in air flow. On the parts a greenish, strongly iridescent layer had formed which later on turned out to be comprised of zinc/chromium oxide. In the corrosion test in the salt spray cabinet according to DIN 50021 SS it was surprisingly found that the chromate layer formed presented a spectacular corrosion protection until the appearance of first corrosion products of 1000 h according to DIN 50961 Chapter 10, in particular Chapter 10.2.1.2.

15 The novel greenish chromate layer had a layer thickness of approx. 800 nm and was produced by a process not involving any chromium(VI) and could be proven to be chromium(VI)-free.

20 The production method according to Example 1 for the novel, greenish chromium(VI)-free chromation is not very economical for conventional plants due to the relatively high temperature of the process solution. Further theoretical reflections concerning chromium(VI)-free chromate coating and further trials finally resulted in economical production conditions.

#### Theoretical Reflections Concerning Chromium(VI)-Free Chromation

25 Chromate coating of zinc takes place by the formation of a so-called conversion layer on the zinc surface, i.e. the zinc surface chemically reacts with the chromate coating solution and is converted into a chromate layer. The formation of conversion layers is a dynamic process beyond chemical equilibrium. In order to describe the underlying processes, one must therefore employ chemical kinetics. By the especially established kinetic model it was possible to obtain starting points in order to optimise the present invention.

30 45 Conversion layer formation in a chromium(III)-based chromate coating solution may be described by means of two reaction equations:

I Elementary zinc passes into solution due to acid attack:



II and precipitates on the zinc surface as zinc chromium oxide together with chromium(III):



60 65 The kinetic model must encompass differential equations for the concentration developments of Zn<sup>2+</sup>, H<sup>+</sup>, Cr(III) and for the thickness growth of the ZnCrO layer. In the reaction rate starting points it was taken into consideration by inserting the term 1/(1+p<sub>1</sub>·m<sub>ZnCrO</sub>)<sup>2</sup> that Reaction I is increasingly slowed down by the growing passive layer. p<sub>1</sub> is a measure for tightness of the layer.

$$\begin{aligned}
 \frac{dc_{Zn^{2+}}}{dt} &= k_1 \times c_{H^+} / (1 + p_1 \times m_{ZnCrO})^2 - & \text{Reaction I} \\
 &k_2 \times c_{Zn^{2+}} \times c_{Cr(III)} + k_3 \times c_{H^+} \times \tanh(p_2 \times m_{ZnCrO}) + & \text{Reaction II} \\
 &k_T \times (c_{0,Zn^{2+}} - c_{Zn^{2+}}) & \text{Mass transfer} \\
 \frac{dc_{H^+}}{dt} &= -2k_1 \times c_{H^+} / (1 + p_1 \times m_{ZnCrO})^2 + & \text{Reaction I} \\
 &2yk_2 \times c_{Zn^{2+}} \times c_{Cr(III)} - 2yk_3 \times c_{H^+} \times \tanh(p_2 \times m_{ZnCrO}) + & \text{Reaction II} \\
 &k_T \times (c_{0,H^+} - c_{H^+}) & \text{Mass transfer} \\
 \frac{dc_{Cr(III)}}{dt} &= -xk_2 \times c_{Zn^{2+}} \times c_{Cr(III)} + xk_3 \times c_{H^+} \times \tanh(p_2 \times m_{ZnCrO}) + & \text{Reaction II} \\
 &k_T \times (c_{0,Cr(III)} - c_{Cr(III)}) & \text{Mass transfer} \\
 \frac{dm_{ZnCrO}}{dt} &= k_2 \times c_{Zn^{2+}} \times c_{Cr(III)} - k_3 \times c_{H^+} \times \tanh(p_2 \times m_{ZnCrO}) & \text{Reaction II}
 \end{aligned}$$

The term  $\tanh(p_2 \times m_{ZnCrO})$  represents the indispensable precondition of reverse reaction II, namely the presence of  $ZnCrO$ . The  $\tanh$  function provides for a smooth transition from 0 to 1, which may be adjusted with  $p_2$ . The differential equation system was resolved numerically by means of a computer. As a result, the layer thickness developments and the concentration developments over time were obtained. As starting values for time  $t_0=0$  there were employed:

$$\begin{aligned}
 c_{0,Zn^{2+}} &= 0 \\
 c_{0,H^+} &= 10-2 \text{ mol/l} & \text{(pH2)} \\
 c_{0,Cr(III)} &= 0.5 \text{ mol/l} \\
 m_{0,ZnCrO} &= 0
 \end{aligned}$$

In FIG. 38 the layer thickness developments for various values of the rate constant  $k_j$  are represented. For good corrosion protection, the passive layer should have maximum possible thickness and at the same time compactness.

FIG. 38 shows a computer simulation of the kinetic model for chromate coating of zinc for various rate constants.

The faster the initial dissolution of zinc (rate constant  $k_1$ ) is and the faster the dissolved zinc precipitates with the chromium(III) (rate constant  $k_2$ ), the thicker the chromate layer will become. Layer growth is strongly favored by the presence of zinc already dissolved in the bath, which fact resulted from simulations with  $c_{0,Zn^{2+}} > 0$ . A lower pH value favors dissolution of zinc but also brings about increased redissolution of the layer.

Based on the model, basically two demands may be established for producing a maximum possible thickness chromate layer. Reaction I and forward reaction II must take place as rapidly as possible, the reverse reaction II must remain slow. In this sense, there result the following starting points:

Reaction I

a pH optimisation

b Avoiding carrying over of inhibitors from the zinc bath

c Addition of oxidants for accelerating zinc dissolution

d Acceleration of zinc dissolution by formation of galvanic elements

Forward reaction II

e The rate constant  $k_2$  should be as high as possible. Chromium(III) complexes generally have slow kinetics. By using suitable ligands it should be possible to accelerate the reaction rate.

f Upon use of further transition metal cations in the chromate coating solution there also result i.a. higher rate constants

than for Cr(III). Moreover these transition metal cations may act as catalysts in ligand replacement on chromium (III).

Reverse reaction III

g Insertion of poorly redissolvable hydroxides, e.g. nickel, cobalt and/or copper hydroxide.

Serial investigations were carried out. Starting points a and b are known to the skilled person.

Acceleration of zinc dissolution via points c and d did also result in thick coatings, however yellowish ones having a chromium/zinc ratio of 1:4 to 1:3, which only afforded low corrosion protection. It was found that good corrosion protection values may only be obtained at chromium/zinc ratios above 1:2.

A higher chromium/zinc ratio at concurrently thicker chromate layers is obtained when the rate constant  $k_2$  (starting point e) is raised, or the forward reaction II is accelerated. After the inventors of the present application had realised that hot chromium(III) solutions result in surprising passive layers, there are the following possibilities in connection with the inventors' theoretical reflections:

Raising the temperature of the chromate coating solution and/or of the partial surface

Raising the chromium(III) concentration in the process solution

Acceleration of ligand replacement kinetics at the chromium(III).

Herefor one should know that chromium(III) in aqueous solutions is essentially present in the form of hexagonal complexes generally having high kinetic stability, and moreover that ligand replacement is the step determining the rate in forward reaction II. By the selection of suitable complex ligands, with which the chromium(III) forms kinetically less stable complexes,  $k_2$  is accordingly increased.

Addition of elements having a catalytic effect on ligand replacement into the chromate coating solution.

In serial investigations chelate ligands (such as di- and tricarboxylic acids as well as hydroxydi- and hydroxytricarboxylic acids) as such forming kinetically less stable complexes with chromium(III), whereas the fluoride complexes are kinetically very stable. When using only such chelate ligands for complexing the chromium(III) and omitting fluoride in the passivation solution, excellent results were obtained even at a treatment temperature of only 60° C., as is shown by Examples 2 and 3.

## EXAMPLE 2

Electrolytically bright-zinc coated (15 m) steel parts were immersed in an aqueous chromate coating solution containing:

50 g/l  $\text{CrCl}_3 \cdot 6 \text{ H}_2\text{O}$  (trivalent chromium salt)

100 g/l  $\text{NaNO}_3$

31.2 g/l malonic acid

the pH of which had previously been adjusted to 2.0 with sodium hydroxide solution. The immersion time was 60 s. Following rinsing and drying there resulted in the salt spray cabinet according to DIN 50021 SS a corrosion protection of 250 h until first attack according to DIN 50961.

Malonic acid is a ligand enabling more rapid ligand replacement kinetics at the chromium(III) than the fluoride of Example 1. Good corrosion protection by far exceeding the minimum requirement of DIN 50961 for Method Group C (yellow chromation) may thus already be achieved at 60° C.

## EXAMPLE 3

Electrolytically bright-zinc coated (15 m) steel parts were immersed in an aqueous chromate coating solution consisting of:

50 g/l  $\text{CrCl}_3 \cdot 6 \text{ H}_2\text{O}$  (trivalent chromium salt)

3 g/l  $\text{Co}(\text{NO}_3)_2$

100 g/l  $\text{NaNO}_3$

31.2 g/l malonic acid

previously adjusted to pH 2.0 with sodium hydroxide solution. Immersion time was 60 s. Following rinsing and drying there resulted in the salt spray cabinet according to DIN 50021 SS a corrosion protection of 350 h until first attack according to DIN 50961.

Cobalt is an element which was capable, in accordance with the model concept, of catalysing ligand replacement and moreover reducing reverse reaction II owing to insertion of kinetically stable oxides into the chromate layer, so that the chromate layer altogether should become thicker. In this point, as well, the model concept established for the present invention is verified under practical conditions. Corrosion protection could once more clearly be enhanced in comparison with Example 3 by nothing but the addition of cobalt into the chromate coating solution.

Novel greenish chromate layers on zinc were produced in analogy with Example 2 at 40, 60, 80 and 100° C. The layer thicknesses of the respective chromate layers were determined by RBS (=Rutherford-Backscattering) testing. In the Table the corresponding corrosion protection values in hours of salt spray cabinet according to DIN 50021 SS until first attack according to DIN 50961 Chapter 10 are additionally listed.

| J/° C. | thickness/nm | Corr. Prot./h |
|--------|--------------|---------------|
| 40     | 100          | 50–60         |
| 60     | 260          | 220–270       |

-continued

|   | J/° C. | thickness/nm | Corr. Prot./h |
|---|--------|--------------|---------------|
| 5 | 80     | 400          | 350 450       |
|   | 100    | 800          | 800–1200      |

Depending on the complex ligands used, which is malonate in Examples 2 and 3, it is partly possible to achieve even considerably higher layer thicknesses and corrosion protection values. By complex ligands containing as the complexing functional group nitrogen, phosphorus or sulfur, ( $-\text{NR}_2$ ,  $-\text{PR}_2$  wherein R independently is an organic, in particular aliphatic radical and/or H, and/or  $-\text{SR}$ , wherein R is an organic, in particular aliphatic radical or H,), it is possible to even produce the indicated layer properties within limits at room temperatures.

## EXAMPLE 4

Steel parts electrolytically coated with a zinc/iron alloy (0.4–0.6% iron) were immersed at 60° C. in the following aqueous chromate coating solution:

25 50 g/l  $\text{CrCl}_3 \cdot 6 \text{ H}_2\text{O}$

100 g/l  $\text{NaNO}_3$

31.2 g/l malonic acid

30 The solution was beforehand adjusted to pH 2.0 with NaOH. Immersion time was 60 s. Following rinsing and drying a transparent, greenish, slightly grey, strongly iridescent layer was visible on the zinc/iron. In the salt spray cabinet in accordance with the above specified DIN and 35 ASTM standards there resulted a corrosion protection of 360 h until first attack according to DIN 50961.

## EXAMPLE 5

40 Steel parts electrolytically coated with a zinc/nickel alloy (8–13% nickel) were immersed at 60° C. into the following aqueous chromate coating solution:

45 50 g/l  $\text{CrCl}_3 \cdot 6 \text{ H}_2\text{O}$

100 g/l  $\text{NaNO}_3$

31.2 g/l malonic acid

50 The solution was beforehand adjusted to pH 2.0 with NaOH. Immersion time was 60 s. Following rinsing and 55 drying a transparent, greenish, dark-grey, strongly iridescent layer was visible on the zinc/nickel. In the salt spray cabinet in accordance with the above specified DIN and ASTM standards there resulted a corrosion protection of 504 h until first attack according to DIN 50961.

55 The novel greenish chromium(VI)-free chromate layer accordingly depending on the production temperature has a thickness of between 100 and 1000 nm, has a weakly green 60 inherent color and a red-green iridescent coloring. The chromate coating solution consists of trivalent chromates, moreover of conducting salts and mineral acids. Application of the chromate coating solutions is generally performed at temperatures above 40° C. The corrosion protection of unmarred greenish chromium(VI)-free chromate coatings depending on the production temperature amounts to 65 100–1200 h in the salt spray cabinet according to DIN 50021 SS until the first appearance of corrosion products. Thus the novel chromation satisfies the minimum requirements to

## 13

corrosion protection for Method Groups C and D according to DIN 50961 (Chapter 10, Table 3), i.e. without chromium (VI) either in production or in the product.

By the present invention it is for the first time made possible to provide chromium(VI)-free conversion layers or passive layers on the basis of chromium(III), which do, however, furnish the corrosion protection of yellow chromations customary in the prior art—i.e., of chromium(VI)-containing passive layers.

This is a singular novelty in the entire galvanisation industry.

Hitherto on a chromium(III) basis only clear to blue layers, referred to as “blue passivation” in technical circles, were known which are variously applied practically.

Moreover yellowish-transparent layers with an addition of cerium are known which are, however, not used practically owing to the very costly cerium addition and their poor corrosion protection properties.

Moreover powdery-greenish layers are known for which the applicant—one of the leading enterprises in the field of surface technology—is not aware of any practical applications.

Even the difference in terms of color of the conversion layers of the present invention is conspicuous in FIG. 1, wherein three treatment methods were performed on zinc-plated screws.

The left-hand pile of screws in accordance with the illustration of FIG. 1 was subjected to a classical blue chromation in accordance with the standard of Method Group B according to DIN 50961 Chapter 10 table 3.

The right-hand pile of screws on the photograph according to FIG. 1 was subjected to a conventional yellow chromation in accordance with the standard of Method Group C according to DIN 50961 Chapter 10 table 3.

The center pile of screws shows the result of passivation of the screws by means of the method in accordance with the invention.

This is consequently a greenish-iridescent, transparent conversion layer, or passive layer.

Moreover the colors represented in FIG. 1 are the true colors, which can be seen from the fact that a color plate and moreover a grey wedge was jointly photographed for the purpose of neutral color representation.

As can be seen from the white test field “White” and from the corresponding field having the density “0.00” from the grey wedge, both test fields are pure white, making evident the neutral filtering and the resulting realistic color representation.

In FIG. 2 scanning electron microscope (SEM) images of the conversion layers of a yellow chromation and of a blue chromation in accordance with the prior art are shown in comparison with the “chromitation” of the present invention.

The layer samples are derived from the correspondingly passivated zinc-plated iron screws shown in FIG. 2, lower half.

The samples treated in accordance with the invention (by “chromitation”) presented a chromium(VI)-free conversion layer having a thickness of approx. 300 nm. In the photographs of FIG. 2 it should be considered that the layers were photographed in a viewing angle of approx. 40°, resulting in foreshortening by approx.  $\cos(40^\circ)=0.77$ .

Based on the SEM images of the chromitation layer of the invention it therefore results that conversion layer thicknesses like in yellow chromation are obtained, however with the difference that the conversion layer of the invention does not contain any toxic chromium(VI).

## 14

The color photograph of FIG. 3 moreover shows the bandwidth of the iridescent coloring of the passive layer according to the invention under practical conditions.

It can already be seen in the photographs of FIGS. 1 and 3 that the passive layer according to the invention does not contain any chromium(VI) ions as it lacks the typically yellow color (cf. right-hand pile of screws of the color photograph of FIG. 1).

Objects according to the photograph of FIGS. 1 and 3 as well as zinc-plated steel sheets passivated by the method of the invention were tested in the salt spray cabinet according to DIN50021SS or ASTM B 117-73, respectively, until the occurrence of first corrosion products according to DIN50961 Chapter 10. Herein it was surprisingly found that the passive layers of the present invention, and thus the objects passivated by the present method, fulfilled the corrosion protection of chromium(VI) passivations, i.e. yellow chromations, although not containing any chromium(VI).

It is worth mentioning that a typical yellow chromation of the prior art affords resistance for approx. 100 hours of exposure to saltwater in accordance with the above specified DIN or ASTM standard, whereas even the tenfold corrosion protection was achieved by the passive layers of the present invention.

The layers of the present invention as well as the methods for producing this layer, or the method for passivation of metal surfaces, thus satisfy the long-standing demand in this technical field for conversion layers doing without any toxic and carcinogenic chromium(VI) compounds while nevertheless even presenting and generally even excelling the corrosion protection of yellow chromations.

EP 00 34 040 A1 does describe a multitude of layers, wherein the colorations of the larger group thereof (produced under the standard conditions set forth by Barnes/Ward) are not specified, however which are referred to as clear. Two examples, i.e. Nos. 16 and 17, describe a greenish, borate-containing layer referred to as cloudy-dull to non-transparent.

Example 14 describes a layer affording a corrosion protection of no more than 4 hours.

In Example 15 of EP 00 34 040, an aluminum-containing layer is described which attains a corrosion protection of 100 hours. This is achieved—in comparison with the remaining examples—merely by the corrosion protection additive aluminum which is lacking in the present invention. Aluminum-free layers of identical or similar baths do, however, only present poor corrosion protection. The layer according to the invention offers significantly higher corrosion protection, namely up to 1000 h, even without this addition.

Examples 16 and 17 describe layers affording a corrosion protection of 300 and 200 hours in the salt spray test and thus in the range claimed by the applicant. Description page 19, line 7 sets forth that layers of more than 1000 nm are required for good corrosion protection. It is thus understandable that these layers, without exception moreover produced from solutions containing boric acid, are described to be cloudy and rather non-transparent (page 14, line 10). The enhanced corrosion protection, in accordance with page 15, lines 1–5, is due to the insertion of borate-containing species.

The layer according to the invention, on the other hand, also offers high (and even higher) corrosion protection without this addition.

There is, however, another difference that is relevant in terms of patent law as well as in practical application: namely, the layers described in Examples 16 and 17 of EP

00 34 040 are soft and come off when wiped and consequently require some sort of hardening process as an after-treatment (page 17, lines 12–21).

The present layers according to the invention are hard and resistant to wiping even without a hardening process, and adhere well. Corrosion protection layers which come off when wiped and which do not adhere to the substrate are useless for practical application.

Furthermore, the layer according to the invention can serve as a basis or substrate for further inorganic and/or organic layers.

In FIG. 4, a photograph is shown as a comparison example. This photograph represents the result of comparison tests carried out by the applicant in comparison with EP 00 34 040. In particular the applicant reproduced the Examples 16 and 17 given in this prior art. Herein steel sheets were immersed into the solutions described in Examples 16 and 17 of EP 00 34 040 and the respective treatment times were observed. FIG. 4 shows the layers on the substrate surfaces obtained in accordance with the prior art, namely from the top to the bottom the first and second sheets successively treated by immersion.

The photograph of FIG. 4 shows from the left to the right in the top half of the illustration a cloth whereby the layer produced in accordance with Example 16—prior art—was wiped, a zinc-plated steel sheet treated in accordance with Example 16, beside it a zinc-plated steel sheet treated in accordance with Example 17—prior art—and on the extreme right also a cloth whereby the layer of Example 17 was wiped. In the second line on the left side—beside the indication of Example 16 and beside it to the right (beside the indication of Example 17) a respective zinc-plated steel sheet coated in accordance with the prior art is shown. What is visible is a milky, white-greenish powdery coating which already comes off when wiped with a soft cloth even without application of particular pressure (see FIG. 4, top half of illustration). The prior art itself suggests that this layer is not a compact oxide zinc/chromium conversion layer firmly adhering to the substrate sheet but a loosely overlying coating substantially consisting of chromium hydroxide. The pH for this coating must be so high that the precipitation limit for chromium hydroxides is already exceeded (page 26, line 12 of EP 0034 040). Precipitation of chromium hydroxide is kinetically inhibited and is favored by immersion of a more or less rough surface. The fact that the layer formation mechanism has to be a different one from the other examples may also be seen from the circumstance that with (Example 16 prior art) or without (Example 17) complexing agents more or less the same result was achieved. In practical reproduction of Examples 16 and 17 of the prior art it was moreover found that the layer became thicker, softer and more powdery with an increasing number of metal sheets coated in the solution. In addition, more and more chromium hydroxide precipitated, whereby the useful life of such a coating solution is limited to a few hours. The layer according to the invention, on the other hand, is produced only from suitable “rapid” complexes and furthermore in a distinctly acidic pH range. The solution is stable over months, presumably even years.

The measurements underlying FIGS. 5 to 36 were performed with a glow-discharge spectrometer.

The element F and die anions could not be analysed by this method. O, H, Cl and K could not be quantified.

The following Table shows the concentration ranges for which calibration is valid:

| Element | Concentration min. in | Concentration max. in |
|---------|-----------------------|-----------------------|
| C       | 0.0067                | 3.48                  |
| S       | 0.0055                | 0.168                 |
| Cr      | 0.0001                | 99.99                 |
| Ni      | 0.0001                | 99.99                 |
| Co      | 0.0001                | 7.00                  |
| Zn      | 0.0001                | 99.99                 |
| Na      | 0.0001                | 0.0068                |
| N       | 0.0001                | 6.90                  |
| B       | 0.0001                | 0.040                 |
| Fe      | 0.0005                | 99.91                 |

15 Sample allocation in FIGS. 5 to 36 results from the following Table:

| Sample No. | Coating                       | Conditions              | Measurement point |
|------------|-------------------------------|-------------------------|-------------------|
| 1          | Chromitaton on Zn (invention) | 60° C., 1 min, pH 2     | A                 |
| 2          |                               | 60° C., 2 min, pH 2     | B                 |
| 3          |                               | 60° C., 1 min, pH 2.5   | A                 |
| 4          |                               | 60° C., 1.5 min, pH 2.5 | A                 |
| 5          |                               | 60° C., 2 min, pH 2.5   | A                 |
| 6          |                               | 100° C., 1 min, pH 2    | A                 |
|            |                               |                         | B                 |
|            |                               |                         | C                 |
|            |                               |                         | D                 |
| 7          | Chromitaton on Zn/Fe          | 60° C., 1 min, pH 2     | A                 |
| 8          | Blue chromation on Zn         | 20° C., 30 s, pH 1.8    | B                 |
| 9          | Yellow chromation on Zn       | 20° C., 45 s, pH 1.8    | A                 |
|            |                               |                         | B                 |

40 FIG. 37 shows a Table containing the evaluations of the depth profile measurements, which indicates that all of the (chromitaton) layers of the invention have thicknesses exceeding 100 nm

What is claimed is:

45 1. A conversion layer comprising chromium(III), said conversion layer being chromium(VI)-free, said conversion layer being a substantially coherent conversion layer on zinc or a zinc alloy, wherein even in the absence of silicate, cerium, aluminum and borate said conversion layer presents a corrosion protection of about 100 to 1000 h in the salt spray test according to DIN 50021 SS or ASTM B 117-73 until first attack according to DIN 50961 Chapter 10; said conversion layer being hard and resistant to wiping.

50 2. A conversion layer according to claim 1, wherein said conversion layer has across the conversion layer thickness a chromium content greater than about 1%, in relation to zinc and chromium in the conversion layer and an average chromium content of more than about 5%; said conversion layer further having a chromium-rich zone with greater than about 20% chromium, in relation to zinc and chromium in the conversion layer, said chromium rich zone having a thickness of more than about 15 nm.

55 3. A conversion layer according to claim 1, further comprising additional components selected from the group consisting of: silicate, cerium, aluminum and borate; additional metal compounds; anions; polymers; corrosion inhibitors; silicic acids; surfactants; diols; triols; polyols; organic acids; amines; plastics dispersions; dyes; pigments; chromogenic agents; amino acids; siccatives; dispersing agents; and mixtures thereof.

## 17

4. A conversion layer according to claim 1, said conversion layer being a basis for further inorganic and/or organic layers.

5. A conversion layer according to claim 1, further comprising a dye or color pigment for modification of the color thereof.

6. A conversion layer according to claim 1, having a thickness of about 100 nm.

7. A conversion layer according to claim 1, said layer being free from the presence of silicate, cerium, aluminum, and borate.

8. A conversion layer according to claim 1, said layer having a layer thickness of about 100 nm to 1000 nm, said conversion layer having across the conversion layer thickness a chromium content of greater than 1% based upon zinc and chromium.

9. A conversion layer according to claim 1, said layer being clear or substantially colorless.

10. A conversion layer according to claim 1, said layer further comprising cobalt.

11. A conversion layer according to claim 1, said layer further comprising one or more metal compounds selected from the group consisting of 1- to 6-valent metal compounds.

12. A conversion layer according to claim 1, said layer further comprising one or more anions.

13. A conversion layer according to claim 1, having a chromium index greater than 10, the chromium index being defined as the average chromium content in said conversion layer greater than 1% chromium, multiplied by the thickness of said conversion layer.

14. A conversion layer according to claim 3, wherein said anions include an anion selected from the group consisting of halide ions, sulfurous ions, nitrate ions, phosphoric ions, diphosphate ions, linear and/or cyclic oligophosphate ions, linear and/or cyclic polyphosphate ions, hydrogen phosphate ions, carboxylic acid anions, and silicon-containing anions.

15. A conversion layer according to claim 3, wherein said additional metal compounds include at least one 1- to 6-valent metal compound selected from the group consisting of compounds of Na, Ag, Al, Co, Ni, Fe, Ga, In, lanthanides, Zr, Sc, Ti, V, Cr, Mn, Cu, Zn, Y, Nb, Mo, Hf, Ta, W.

16. A conversion layer according to claim 1, said conversion layer being transparent.

17. A conversion layer according to claim 1, said conversion layer being iridescent.

18. A conversion layer according to claim 1, said conversion layer having a chromium-rich zone comprising greater than about 20% chromium based on zinc and chromium in said chromium-rich zone.

19. A conversion layer according to claim 18, said chromium-rich zone having a thickness of at least 15 nm.

20. A conversion layer according to claim 1, said conversion layer being clear, transparent and essentially colorless, said conversion layer presenting a multi-colored iridescence.

21. A conversion layer according to claim 1, said conversion layer having a thickness of about 100 nm to 1000 nm.

22. A conversion layer according to claim 1, said chromium(III) being provided via a chromium(III) complex having ligand replacement kinetics more rapid than the fluoride replacement kinetics in chromium(III)-fluorocomplexes.

23. A method for producing a chromium(VI)-free conversion layer affording at least the corrosion protection of conventional chromium(VI)-containing yellow chromations, wherein a metallic surface is treated with a solution of at least one chromium(III) complex and at least

## 18

one salt; said chromium(III) complex having ligand replacement kinetics more rapid than the fluoride replacement kinetics in chromium(III)-fluorocomplexes; chromium(III) being present in said solution in a concentration of 5 to 100 g/l, said method producing a chromium(VI)-free conversion layer.

24. A method according to claim 23, wherein treatment is carried out at 20 to 100° C.

25. A method according to claim 23, wherein ligands of the chromium(III) complex are selected from the group consisting of: chelate ligands, and complex ligands having a complexing functional group containing nitrogen, phosphorus or sulfur.

26. A method according to claim 23, said metal surface being zinc or a zinc alloy.

27. A method according to claim 25, claim 25, said chelate ligands being selected from the group consisting of dicarboxylic acids, tricarboxylic acids, hydroxycarboxylic acids, maleic acid, phthalic acid, terephthalic acid, tartaric acid, citric acid, malic acid, ascorbic acid, acetylacetone, urea, urea derivatives, and mixtures thereof.

28. A method according to claim 25, said complex ligands being selected from the group consisting of —NR<sub>2</sub>, —PR<sub>2</sub>, and —SR compounds, wherein R is H or an organic radical, phosphinates, phosphinate derivatives, and mixtures thereof.

29. A method according to claim 24, wherein said treatment is carried out at 30–60° C.

30. A method according to claim 25, wherein said chelate ligands are selected from the group consisting of dicarboxylic acids, tricarboxylic acids and hydroxycarboxylic acids.

31. A method according to claim 25, wherein said chelate ligands are selected from the group consisting of oxalic acid, malonic acid, succinic acid, glutaric acid, adipic acid, pimelic acid, suberic acid, azelaic acid, sebatic acid, maleic acid, phthalic acid, terephthalic acid, tartaric acid, citric acid, malic acid, and ascorbic acid.

32. A concentrate for producing a passivation solution for surfaces of zinc or zinc alloys, said concentrate substantially containing chromium(III) for a passivating component, wherein the chromium(III) is present in the form of at least one complex having ligand replacement kinetics more rapid than the fluoride replacement kinetics in chromium(III)-fluorocomplexes, said concentrate being chromium(VI)-free.

33. A concentrate according to claim 32, wherein the chromium(III) complex is selected from complexes with chromium(III) and at least one ligand selected from the group consisting of: chelate ligands, complex ligands wherein the complexing functional group contains nitrogen, phosphorus or sulfur, phosphinates and phosphinate derivatives, and mixtures thereof, among each other as well as in mixed complexes with inorganic anions and H<sub>2</sub>O, said chelate ligands being selected from the group consisting of dicarboxylic acids, tricarboxylic acids, hydroxycarboxylic acids, acetylacetone, urea, urea derivatives, and mixtures thereof.

34. A concentrate according to claim 32, characterised in that the concentrate is present in solid or liquid form.

35. A concentrate according to claim 32, said concentrate comprising further additives selected from the group consisting of: sealers, dewatering fluids, additional metal compounds, anions, polymers, corrosion inhibitors, silicic acids, surfactants, diols, triols, polyols, organic acids, amines, plastics dispersions, dyes, pigments, chromogenic agents, amino adds, siccatives, dispersing agents, and mixtures thereof.

36. A concentrate according to claim 33, said complexing functional group of said complex ligands being —NR<sub>2</sub>, —R<sub>2</sub>, or —SR wherein R independently is an aliphatic radical or H.

19

37. A concentrate according to claim 35, said metal compounds being selected from the group consisting of 1- to 6-valent metal compounds of Na, Ag, Al, Co, Ni, Fe, Ga, In, lanthanides, Zr, Sc, Ti, V, Cr, Mn, Cu, Zn, Y, Nb, Mo, Hf, Ta, and W; said anions being selected from the group consisting of halide ions, sulfurous ions, nitrate ions, phosphoric ions, carboxylic acid anions, and silicon-containing anions; said polymers being selected from the group consisting of organic polymers.

38. A concentrate according to claim 35, said silicic acids being colloidal or disperse silicic acids, said organic acids being monocarboxylic acids, said chromogenic agents being metallic chromogenic agents, said amino acid being glycine, said siccatives being cobalt siccatives.

39. A passivation bath for passivating a metal surface of zinc, cadmium, aluminum, or alloys thereof among each other and/or with other metals, said bath comprising chromium(III) as a passivating component, wherein chromium(III) is present in a concentration of about 5 to 100 g/l, said bath being effective, upon immersing said metal surface therein, to provide a conversion layer on said metal surface which presents a corrosion protection of about 100 to 1000 h in the salt spray test according to DIN 50021 SS or ASTM B 117-73 until first attack according to DIN 50961 Chapter 10, said passivation bath being chromium(VI)-free.

40. A passivation bath according to claim 39, wherein chromium(III) is present in a concentration of about 5 g/l to 80 g/l.

41. A passivation bath according to claim 39, wherein said bath has a pH between about 1.5 and 3.

42. A passivation bath according to claim 39, wherein said bath contains about 20 g/l chromium(III) and has a pH of about 2 to 2.5.

43. A passivation bath according to claim 39, wherein said bath contains further additives selected from the group consisting of sealers, dewatering fluids additional metal compounds anions, polymers, corrosion inhibitors, silicic acids, surfactants, diols, triols, polyols, organic acids, amines, plastics dispersions, dyes, pigments, chromogenic agents, amino acids, siccatives, dispersing agents, and mixtures thereof.

44. A passivation bath according to claim 39, said bath having a bath temperature of about 20 to 100° C.

45. A passivation bath according to claim 40, wherein said chromium (III) is present in a concentration of about 10 g/l to 30 g/l.

46. A passivation bath according to claim 43, wherein said additional metal compounds are selected from the group consisting of 1- to 6 valent metal compounds of Na, Ag, Al, Co, Ni, Fe, Ga, In, lanthanides, Zr, Sc, Ti, V, Cr, Mn, Cu, Zn, Y, Nb, Mo, Hf, Ta, and W;

said anions being selected from the group consisting of halide ions, sulfurous ions, nitrate ions, phosphoric ions, diphosphate ions, linear and cyclic oligophosphate ions, linear and cyclic polyphosphate ions, hydrogen phosphate ions, carboxylic acid anions, and silicon-containing anions;

said silicic acids being colloidal or disperse silicic acids; said chromogenic agents including metallic chromogenic agents.

47. A passivation bath according to claim 43, said amino acids including glycine.

48. A passivation bath according to claim 43, said additional metal compounds being selected from the group consisting of 1- to 6-valent metal compounds of Na, Ag, Al, Co, Ni, Fe, Ga, In, lanthanides, Zr, Sc, Ti, V, Cr, Mn, Cu, Zn, Y, Nb, Mo, Hf, Ta, and W.

20

49. A passivation bath according to claim 43, said anions being selected from the group consisting of halide ions, sulfurous ions, nitrate ions, phosphoric ions, carboxylic acid anions; and silicon-containing anions.

50. A passivation bath according to claim 39, said chromium(III) being present in said passivation bath at least in part as a chromium(III) complex having ligand replacement kinetics more rapid than the fluoride replacement kinetics in chromium(III)-fluorocomplexes.

51. A method for passivating surfaces of zinc or zinc alloys, comprising the steps of immersing said surface, for an immersion period, in a passivation bath comprising chromium(III) as a passivating component, wherein chromium(III) is present in a concentration of about 5 to 100 g/l, and thereby providing a conversion layer on said surface which presents a corrosion protection of about 100 to 1000 h in the salt spray test according to DIN 50021 SS or ASTM B 117-73 until first attack according to DIN 50961 Chapter 10, wherein both said passivation bath and said conversion layer provided on said surface are chromium(VI)-free.

52. A method according to claim 51, wherein the immersion period is between about 15 and 200 seconds.

53. A method according to claim 51, said method being an elevated-temperature chromate coating method with rinsing water recycling over at least 2 cascaded rinsing stages.

54. A method according to claim 53, characterised in that a blue chromation is performed in one of the rinsing steps.

55. A method according to claim 52, said immersion period being between about 15 and 100 seconds.

56. A method according to claim 51, said chromium(III) being present in said passivation bath at least in part as a chromium(III) complex having ligand replacement kinetics more rapid than the fluoride replacement kinetics in chromium(III)-fluorocomplexes.

57. A conversion layer obtained by a method comprising the steps of immersing a metal surface of zinc or zinc alloy, for an immersion period, in a passivation bath comprising chromium(III) as a passivating component, wherein chromium(III) is present in a concentration of about 5 to 100 g/l, and thereby providing said conversion layer on said metal surface, said conversion layer and said passivation bath each being chromium(VI)-free, said conversion layer presenting a corrosion protection of about 100 to 1000 h in the salt spray test according to DIN 50021 SS or ASTM B 117-73 until first attack according to DIN 50961 Chapter 10.

58. A conversion layer according to claim 57, said conversion layer providing corrosion protection of at least 100 hours in the salt spray test according to DIN 50021 SS until first attack according to DIN 50961 Chapter 10.

59. A conversion layer according to claim 57, said layer presenting a greenish, red-green iridescent color for zinc.

60. A conversion layer according to claim 57, said layer having a layer thickness of about 100 nm.

61. A conversion layer according to claim 57, said chromium(III) being present in said passivation bath at least in part as a chromium(III) complex having ligand replacement kinetics more rapid than the fluoride replacement kinetics in chromium(III)-fluorocomplexes.

62. A conversion layer obtained by a method comprising treating a metallic surface of zinc or zinc alloys with a solution of at least one chromium(III) complex and at least one salt, said chromium(III) complex having ligand replacement kinetics more rapid than the fluoride replacement kinetics in chromium(III)-fluorocomplexes, said solution being chromium(VI)-free.

63. A conversion layer comprising chromium(III), said conversion layer being chromium(VI)-free, said conversion

## 21

layer being a substantially coherent conversion layer on zinc or a zinc alloy, said conversion layer presenting a corrosion protection of about 100 to 1000 h in the salt spray test according to DIN 50021 SS or ASTM B 117-73 until first attack according to DIN 50961 Chapter 10, said conversion layer having an average chromium content of more than approximately 5% based on zinc and chromium, said conversion layer having a chromium index greater than approximately 10, wherein the chromium index is defined as said average chromium content (chromium/(chromium+zinc)) in the layer greater than 1% Cr, multiplied by the layer thickness in nm.

64. A conversion layer according to claim 63, said layer further comprising one or more materials selected from the group consisting of polymers, corrosion inhibitors, silicic acids, surfactants, polyols, organic acids, amines, plastics, dispersions, dyes, pigments, chromogenic agents, amino acids, siccatives, dispersing agents, organic polymers, diols, trids, monocarboxylic acids, carbon black, metal chromogenic agents, glycin, and cobalt siccatives.

65. A conversion layer comprising chromium(III), said conversion layer being chromium(VI)-free, said conversion layer being a substantially coherent conversion layer on zinc or a zinc alloy, said conversion layer having a thickness of about 100–1000 nm, said conversion layer presenting a corrosion protection of about 100 to 1000 h in the salt spray test according to DIN 50021 SS or ASTM B 117-73 until first attack according to DIN 50961 Chapter 10.

66. A conversion layer according to claim 65, wherein said conversion layer has across the conversion layer thickness a chromium content greater than about 1%, in relation to zinc and chromium in the conversion layer and an average chromium content of more than about 5%.

67. A conversion layer according to claim 65, having a thickness of about 100 nm.

## 22

68. A conversion layer according to claim 65, further comprising a dye or color pigment for modification of the color thereof.

69. A conversion layer according to claim 65, said layer being free from the presence of silicate, cerium, aluminum, and borate.

70. A conversion layer according to claim 65, said layer being clear or substantially colorless.

71. A conversion layer according to claim 65, said layer further comprising cobalt.

72. A conversion layer according to claim 65, said layer further comprising one or more metal compounds selected from the group consisting of 1- to 6-valent metal compounds.

73. A conversion layer according to claim 65, said layer further comprising one or more anions.

74. A conversion layer according to claim 65, having a chromium index greater than 10, the chromium index being defined as the average chromium content (chromium/(chromium+zinc)) in said conversion layer greater than 1% chromium, multiplied by the thickness in nm of said conversion layer.

75. A conversion layer according to claim 65, said conversion layer being transparent.

76. A conversion layer according to claim 65, said conversion layer being iridescent.

77. A conversion layer according to claim 65, having a chromium(III) being provided via a chromium(III) complex having ligand replacement kinetics more rapid than the fluoride replacement kinetics in chromium(III)-fluorocomplexes.

78. A conversion layer according to claim 65, said conversion layer having a chromium-rich zone with greater than about 20% chromium, in relation to zinc and chromium in the conversion layer.

\* \* \* \* \*

UNITED STATES PATENT AND TRADEMARK OFFICE  
**CERTIFICATE OF CORRECTION**

PATENT NO. : 6,946,201 B2  
APPLICATION NO. : 09/904993  
DATED : September 20, 2005  
INVENTOR(S) : Patricia Preikschat et al.

Page 1 of 6

It is certified that error appears in the above-identified patent and that said Letters Patent is hereby corrected as shown below:

Title Page

(\*) Notice:, after “days.”, please insert --This patent is subject to a terminal disclaimer--.

(63) Related U.S. Application Data, after “filed”, please delete “as.....6,287,704” and insert therefor

--3/29/1999, now U.S. Pat. No. 6,287,704, which is a 371 of PCT/DE97/00800 filed 4/18/1997--. Other Publications, “Kinetics.....1581.”, line 2, after “Cr3”, please delete “0” and insert therefor --O--.

Title Page 2

Other Publications, “Database.....Zusammenfussung.”, line 2, after “GB;”, please insert --Class E31,--.

Other Publications, “Patricia Preikschat.....1-10.”, line 1, please delete “Udner” and insert therefor --Under--.

Drawings

The sheets of drawings consisting of figures 1-4, should be deleted to appear as per attached figs. 1-4,

Specification

Column 8, line 63, please delete “ $1/(1+p_1 \cdot m_{ZnCrO})^2$ ” and insert therefor -- $1/(1+p_1 \cdot m_{ZnCrO})^2$ --.

Column 9, line 5, after “(C”, please delete “ $_{OZn}^2$ ”, and insert therefor -- $_{OZn}^2$ --.

Column 9, line 20, please delete “ $P_2 \times m_{ZrO}$ ” and insert therefor -- $p_2 \times m_{ZnCrO}$ --.

Claim 27

Line 1, after “claim 25,”, please delete --claim 25,--.

UNITED STATES PATENT AND TRADEMARK OFFICE  
**CERTIFICATE OF CORRECTION**

PATENT NO. : 6,946,201 B2  
APPLICATION NO. : 09/904993  
DATED : September 20, 2005  
INVENTOR(S) : Patricia Preikschat et al.

Page 2 of 6

It is certified that error appears in the above-identified patent and that said Letters Patent is hereby corrected as shown below:

Claim 46

Line 14, please delete “a gents” and insert therefor --agents--.

Claim 65

Line 6, please delete “In” and insert therefor --in--.

Claim 77

Line 1, after “claim”, please insert --65,--.

Signed and Sealed this

Thirtieth Day of January, 2007

A handwritten signature in black ink, appearing to read "Jon W. Dudas", is centered within a dotted rectangular box.

JON W. DUDAS  
*Director of the United States Patent and Trademark Office*

U.S. Patent

Sep. 20, 2005

Sheet 1 of 38

6,946,201 B2



**Fig. 1**

U.S. Patent

Sep. 20, 2005

Sheet 2 of 38

6,946,201 B2



**Fig. 2**

U.S. Patent

Sep. 20, 2005

Sheet 3 of 38

6,946,201 B2



**Fig. 3**

U.S. Patent

Sep. 20, 2005

Sheet 4 of 38

6,946,201 B2



**Fig. 4**



US006946201C1

**(12) EX PARTE REEXAMINATION CERTIFICATE (6017th)**  
**United States Patent**  
**Preikschat et al.**

(10) Number: **US 6,946,201 C1**  
(45) Certificate Issued: **Nov. 20, 2007**

**(54) CHROMIUM (VI)-FREE CONVERSION LAYER AND METHOD FOR PRODUCING IT**

**(75) Inventors:** **Patricia Preikschat**, Trebur (DE); **Rolf Jansen**, Trebur (DE); **Peter Hulser**, Trebur (DE)

**(73) Assignee:** **SurTec International GmbH**, Zwingenberg (DE)

**Reexamination Request:**

No. 90/007,778, Oct. 25, 2005

**Reexamination Certificate for:**

Patent No.: **6,946,201**  
Issued: **Sep. 20, 2005**  
Appl. No.: **09/904,993**  
Filed: **Jul. 13, 2001**

**Related U.S. Application Data**

**(63) Continuation of application No. 09/171,558, filed as application No. PCT/DE97/00800 on Apr. 18, 1997, now Pat. No. 6,287,704.**

**(30) Foreign Application Priority Data**

Apr. 19, 1996 (DE) ..... 196 15 664

**(51) Int. Cl.**

**C23C 22/05** (2006.01)  
**C23C 22/53** (2006.01)

**(52) U.S. Cl.** ..... **428/472.1; 428/628; 428/629; 428/632; 428/658; 428/659; 148/247; 148/251; 148/258; 148/265; 148/267; 148/268; 148/273; 148/274; 148/283; 148/284**

**(58) Field of Classification Search** ..... None  
See application file for complete search history.

**(56) References Cited**

**U.S. PATENT DOCUMENTS**

2,035,380 A 3/1936 Wilhelm  
2,035,385 A 3/1936 McLean  
2,106,904 A 2/1938 Wilhelm

|             |         |                  |
|-------------|---------|------------------|
| 2,559,878 A | 7/1951  | Johnson          |
| 2,563,431 A | 8/1951  | Spruance, Jr.    |
| 2,620,265 A | 12/1952 | Hesch            |
| 2,904,413 A | 9/1959  | Hampel           |
| 3,072,516 A | 1/1963  | Bellinger et al. |
| RE26,130 E  | 12/1966 | Bellinger et al. |
| 3,382,111 A | 5/1968  | Tongyai et al.   |
| 3,477,882 A | 11/1969 | Coulman          |
| 3,553,034 A | 1/1971  | Harvey et al.    |
| 3,556,868 A | 1/1971  | Ziemba           |
| 3,787,326 A | 1/1974  | Deyrup           |
| 3,843,430 A | 10/1974 | Kinder           |
| 3,857,739 A | 12/1974 | Prust et al.     |
| 3,900,689 A | 8/1975  | Deyrup           |
| 3,932,198 A | 1/1976  | Schneider        |
| 4,126,490 A | 11/1978 | Aoki             |

(Continued)

**FOREIGN PATENT DOCUMENTS**

|    |         |         |
|----|---------|---------|
| DE | 2166737 | 6/1975  |
| DE | 2900099 | 10/1979 |
| DE | 3038699 | 7/1981  |

(Continued)

**OTHER PUBLICATIONS**

DIN 50 961, Ch. 10, "Prüfung des Chromatierüberzuges" (English Title "Testing of Chromate Conversion Coatings"), Jun. 1987 (with English translation).

(Continued)

*Primary Examiner*—Stephen Stein

**(57) ABSTRACT**

A chromium(VI)-free, chromium(III)-containing and substantially coherent conversion layer on zinc or zinc alloys presenting, even in the absence of further components such as silicate, cerium, aluminum and borate, a corrosion protection of approx. 100 to 1000 h in the salt spray test according to DIN 50021 SS or ASTM B 117-73 until first attack according to DIN 50961 Chapter 10; being clear, transparent and substantially colorless and presenting multi colored iridescence; having a layer thickness of approx. 100 nm to 1000 nm; and being hard, adhering well and being resistant to wiping.



Computer simulation of the kinetic model of chromate coating of zinc for various rate constants

## U.S. PATENT DOCUMENTS

|              |         |                  |
|--------------|---------|------------------|
| 4,141,758 A  | 2/1979  | Glassman et al.  |
| 4,169,741 A  | 10/1979 | Lampazer et al.  |
| 4,171,231 A  | 10/1979 | Bishop et al.    |
| 4,263,059 A  | 4/1981  | Guhde et al.     |
| 4,298,404 A  | 11/1981 | Greene           |
| 4,349,392 A  | 9/1982  | Huvar            |
| 4,359,345 A  | 11/1982 | DaFonte, Jr.     |
| 4,359,346 A  | 11/1982 | DaFonte, Jr.     |
| 4,359,347 A  | 11/1982 | DaFonte, Jr.     |
| 4,359,348 A  | 11/1982 | Crotty           |
| 4,367,099 A  | 1/1983  | Lash et al.      |
| 4,384,902 A  | 5/1983  | Crotty et al.    |
| 4,444,601 A  | 4/1984  | Greene           |
| 4,539,348 A  | 9/1985  | Gajria et al.    |
| 4,578,122 A  | 3/1986  | Crotty           |
| 4,702,802 A  | 10/1987 | Umino et al.     |
| 4,705,576 A  | 11/1987 | Klos et al.      |
| 4,749,418 A  | 6/1988  | Saeki et al.     |
| 4,801,337 A  | 1/1989  | Higgins          |
| 5,091,023 A  | 2/1992  | Saeki et al.     |
| 5,141,575 A  | 8/1992  | Yoshitake et al. |
| 5,230,750 A  | 7/1993  | Shindou et al.   |
| 5,294,266 A  | 3/1994  | Hauffe et al.    |
| 5,368,655 A  | 11/1994 | Klos             |
| 5,393,354 A  | 2/1995  | Bishop           |
| 5,407,749 A  | 4/1995  | Bishop           |
| 5,415,702 A  | 5/1995  | Bishop et al.    |
| 5,807,442 A  | 9/1998  | Goodreau         |
| 5,820,741 A  | 10/1998 | Bibber           |
| 5,876,517 A  | 3/1999  | Jeannier         |
| 6,224,657 B1 | 5/2001  | Myers et al.     |
| 6,287,704 B1 | 9/2001  | Prekschat et al. |
| 6,375,726 B1 | 4/2002  | Matzdorf et al.  |

## FOREIGN PATENT DOCUMENTS

|    |         |         |
|----|---------|---------|
| DE | 3423990 | 1/1985  |
| DE | 3213384 | 1/1991  |
| DE | 4135524 | 4/1993  |
| EP | 034040  | 8/1981  |
| EP | 337411  | 10/1989 |
| GB | 1461244 | 1/1977  |
| GB | 2097024 | 10/1982 |
| GB | 2144773 | 3/1985  |
| JP | 50-1934 | 1/1975  |
| JP | 61-587  | 1/1986  |
| RU | 1781316 | 12/1992 |

## OTHER PUBLICATIONS

- “Some Metal Derivatives of Azo and Azomethine Dyes,” Journal of the American Chemical Society, vol. 74, No. 14, pp. 3461 and 3509–3512, Jul. 20, 1952.
- PCT International Search Report for PCT International Application PCT/DE97/00800, Sep. 5, 1997.
- Dr.-Ing. Uka Handreg and Dipl.-Ing. Stefen Piepenstock, Prüfbericht–Untersuchungen an Blauchromatierungen, pp. 1–4, Jan. 8, 2002.

Von W. Stechelbach, Chromatierrungstechnik an Verzinkten Oberflächen, Galvanotechnik, D–7968 Saulgau, 82 Nr. 8, pp. 2669–2672, 1991.

Zusammenstellung der Experimentellen Daten, Jul. 17, 2002, 9 pages.

SurTec® 660 Dreiwertige Blauchromatierung, Surtec GmbH, Feb. 1994.

SurTec® 662 Dreiwertige Temperbeständige Blauchromatierung, SurTec GmbH, Feb. 1994.

Arthur Schaier, First Request for Reexamination of U.S. Pat. No. 6,287,704 (granted as re-exam U.S. Appl. No. 90/006, 211), Request filed in U.S. Patent Office on Jan. 25, 2002, pp. 1–118.

Arthur Schaier, Submission of Prior Art Under 37 CFR 1.501 filed in re-exam proceeding U.S. Appl. No. 90/006, 211, filed in U.S. Patent Office on Mar. 11, 2002, pp. 1–4. Patricia Prekschat, Declaration of Patricia Prekschat Under Rule 1.132 filed in re-exam proceeding U.S. Appl. No. 90/006,211, dated Dec. 28, 2002, pp. 1–10.

Arthur Schaier, Second Request for Reexamination of U.S. Pat. No. 6,287,704 (granted as re-exam U.S. Appl. No. 90/006,672), filed in U.S. Patent Office on Jun. 20, 2003, pp. 1–25.

Sudha Damji, Declaration of Sudha Damji and attached Exhibit A, dated Jun. 18, 2003 (submitted with the second request for reexamination of U.S. Pat. No. 6,287,704) filed in re-exam proceeding U.S. Appl. No. 90/006,672 on Jun. 20, 2003, pp. 1–33.

“Chromate Coating From Trivalent Solution”, Products Finishing, Aug. 1983, pp. 64–65.

Barnes, et al., “Non-Chromate Passivation Treatments for Zinc,” Transactions of the Institute of Metal Finishing, Summer, 1982, pp. 45–48, vol. 60.

Klos, “Clear Chromates: Theory and Practice”, Products Finishing, Jun. 1988, pp. 72–78.

“Kinetics of Formation and Dissociation of [Cr<sub>3</sub>O(O<sub>2</sub>CCH<sub>3</sub>)<sub>6</sub>(urea)<sub>3</sub>]<sup>+</sup>: An Example of Statistically Controlled Kinetics and Equilibrium,” John P. Bourke, et al., Inorganic Chemistry; vol. 35, No. 6, Mar. 13, 1996; pp. 1577–1581.

SurTec® 664 Dreiwertige, Temperbeständige Blauchromatierung Mit Eiseninhibitor, SurTec GmbH, Feb. 1994.

Optische Defizite der Surtec Beispiele 2 and 3 aus dem Patent EP 0907762, at least as early as Jul. 17, 2002.

Chemisch erzeugte Schutzschichten, pp. 470–473, at least as early as Jul. 22, 2002.

Coventya, *Intenal Note*, Subject: Opposition au brevet EP 907762, Jul. 1, 2002, 4 pages.

Peter Hülser, et al., Chromitierung, Mo Metallocberfläche Beschichtungen von Metall Und Kunststoff, Oct. 1996, 5 pages.

**1**  
**EX PARTE**  
**REEXAMINATION CERTIFICATE**  
**ISSUED UNDER 35 U.S.C. 307**

THE PATENT IS HEREBY AMENDED AS  
 INDICATED BELOW.

**Matter enclosed in heavy brackets [ ] appeared in the patent, but has been deleted and is no longer a part of the patent; matter printed in italics indicates additions made to the patent.**

AS A RESULT OF REEXAMINATION, IT HAS BEEN DETERMINED THAT:

The patentability of claims 1–22, 51–61, 63–76 and 78 is confirmed.

Claims 33, 36 and 62 are cancelled.

Claims 23, 26, 27, 32, 39 and 77 are determined to be patentable as amended.

Claims 24, 25, 28–31, 34–35, 37, 38 and 40–50, dependent on an amended claim, are determined to be patentable.

**23.** A method for producing a chromium(VI)-free conversion layer affording at least the corrosion protection of conventional chromium(VI)-containing yellow chromations, wherein a metallic surface *selected from the group consisting of zinc, cadmium and alloys of these metals among each other and/or with iron or other metals* is treated with a solution of at least one chromium(III) complex and at least one salt; said chromium(III) complex having ligand replacement kinetics more rapid than the fluoride replacement kinetics in chromium(III)-fluorocomplexes; chromium (III) being present in said solution in a concentration of 5 to 100 g/l, said method producing a chromium(VI)-free conversion layer *that presents a corrosion protection of about 100 to 1000 h in the salt spray test according to DIN 50021 SS or ASTM B 117-73 until first attack according to DIN 50961 Chapter 10.*

**26.** A method according to claim 23, said metal surface being zinc [or a zinc alloy].

**27.** A method according to [claim 25.] claim 25, said chelate ligands being selected from the group consisting of dicarboxylic acids, tricarboxylic acids, hydroxycarboxylic acids, maleic acid, phthalic acid, terephthalic acid, tartaric acid, citric acid, malic [add] acid, ascorbic acid, acetylacetone urea, urea derivatives, and mixtures thereof.

**32.** A concentrate for producing a passivation solution for surfaces of zinc or zinc alloys, said concentrate substantially containing chromium(III) for a passivating component, wherein the chromium(III) is present in the form of at least one complex having ligand replacement kinetics more rapid than the fluoride replacement kinetics in chromium(III) fluorocomplexes, said concentrate being chromium(VI)-free, wherein the chromium(III) complex is selected from complexes with chromium(III) and at least one ligand selected from the group consisting of: complex ligands wherein the complexing functional group contains nitrogen, phosphorus or sulfur, phosphinates and phosphinate derivatives, and mixtures thereof with chelate ligands, among each other as well as in mixed complexes with inorganic anions and H<sub>2</sub>O, said complexing functional group of said complex ligands being —NR<sub>2</sub>, —R<sub>2</sub>, or —SR wherein R independently is an aliphatic radical or H.

**39.** A passivation bath for [passivating] passivating a metal surface of zinc, cadmium, aluminum, or alloys thereof among each other and/or with other metals, said bath comprising chromium(III) as a passivating component, wherein chromium(III) is present in a concentration of about 5 to 100 g/l, said bath being effective, upon immersing said metal surface therein, to provide a conversion layer on said metal surface which presents a corrosion protection of about 100 to 1000 h in the salt spray test according to DIN 50021 SS or ASTM B 117-13 until first attack according to DIN 50961 Chapter 10, said passivation bath being chromium(VI)-free, said bath having said metal surface immersed therein.

**77.** A conversion layer according to claim 65, said chromium(III) being provided via a chromium(III) complex having ligand replacement kinetics more rapid than the fluoride replacement kinetics in chromium(III)-fluorocomplexes.

\* \* \* \* \*